

May 1, 1934.

N. FRANZEN

1,956,860

SHEET GLASS MANUFACTURE

Filed Oct. 20, 1932

3 Sheets-Sheet 1



INVENTOR-  
*Nicholas Franzen*  
BY  
*Cooper, Kerr, Dunham*  
ATTORNEYS

May 1, 1934.

N. FRANZEN

1,956,860

SHEET GLASS MANUFACTURE

Filed Oct. 20, 1932

3 Sheets-Sheet 2

FIG. 2.



FIG. 3.



INVENTOR-  
*Nicholas Franzen*  
BY  
*Cooper, Keer & Dunham*  
ATTORNEYS

May 1, 1934.

N. FRANZEN

1,956,860

SHEET GLASS MANUFACTURE

Filed Oct. 20, 1932

3 Sheets-Sheet 3



INVENTOR-  
Niklas Franzen  
BY  
Cooper, Kerr, Bunker  
ATTORNEYS

## UNITED STATES PATENT OFFICE

1,956,860

## SHEET GLASS MANUFACTURE

Nicklas Franzen, Long Beach, Calif., assignor to  
 Mississippi Glass Company, New York, N. Y., a  
 corporation of New York

Application October 20, 1932, Serial No. 638,697

9 Claims. (Cl. 49—32)

This invention pertains to the manufacture of sheet glass and the primary object of the invention is to disclose an improved method and apparatus for producing intermittent sheets while maintaining a continuous flow of molten metal from the furnace.

Further and other objects and advantages will be apparent from the specification and claims, and from the accompanying drawings which illustrate what is now considered the preferred embodiment of the invention.

Fig. 1 is a somewhat diagrammatic view of one form of the apparatus.

Fig. 2 is an enlarged detail view of a portion of the apparatus, with the ladle in dumping position.

Fig. 3 is an enlarged view on line 3—3 of Fig. 1.

Fig. 4 is a diagrammatic view of a modified form of the apparatus for making reinforced wire sheets.

In the drawings 10 is the furnace containing molten metal 12. An extension of the furnace 14 is provided with one or more openings 16 through the bottom thereof. A plug 18 is adapted to close each opening at the will of the operator. As illustrated, two circular orifices 16 are provided, but the number and shape of the openings may be varied according to circumstances.

Below the orifices is a semi-cylindrical ladle 20, preferably lined with refractory material 22, and supported for partial rotation on trunnions 24 in bearings 26. Gears 28 on the ends of the trunnions are actuated periodically by racks 30 to tip the ladle at regular intervals of time in order to dump metal from the ladle, as shown in Fig. 2, to form a gob 31 above the forming pass between rolls 32 and 34. Each gob contains enough metal to form a sheet 36 of the desired dimensions. It will be observed that the ladle and tilting device are so arranged that the flow of metal into the ladle is uninterrupted even while the dumping operation is occurring. Briefly, the ladle serves to divide the flowing molten metal into substantially equal batches, and to deliver those batches to the forming pass. After the sheet is formed it passes over apron 38 and rolls 40 to the rear.

A refractory arch 42 may be provided to prevent loss of heat from the metal in the ladle and while the metal is enroute from furnace to ladle, and, if desired, additional heat may be supplied within the arch by burners 44.

In the process of making wire glass the apparatus is modified as in Fig. 4 by providing additional orifices 46 with suitable plugs 48. Metal

flows through openings 46 to a second ladle 50 similar in structure and operation to the apparatus already described, the ladle being so located as to dump its metal between rolls 32 and 52. In operation, ladle 20 supplies metal to be formed by rolls 32—34 into a lower half-sheet, while ladle 50 supplies metal to be formed into the upper half-sheet between rolls 32—52, these latter rolls also serving to weld the two half-sheets together with the wire mesh between them. The wire 54 is supplied from reel 56 and is guided to position by fingers 58 in well known manner.

In the claims of this application, for the sake of clarity, the metal flowing through the orifices 16 is considered to be a single "stream", while the metal from orifices 46 is considered as another "stream".

It is to be understood that the invention is not limited to the specific embodiment herein illustrated and described, but may be used in other ways without departure from its spirit as defined by the following claims.

I claim:

1. In the manufacture of sheet glass, means for maintaining two streams of molten metal, in combination with means operable periodically for dividing each of said streams into batches, two sheet forming passes, means for delivering batches from one of said streams to one of said passes, means for delivering batches from the other of said streams to the other of said passes, and means for combining the sheets formed by the two passes into single sheets.

2. In the manufacture of sheet glass, means for maintaining two streams of molten metal, in combination with means operable periodically for dividing each of said streams into batches, two sheet forming passes, means for delivering batches from one of said streams to one of said passes, means for delivering batches from the other of said streams to the other of said passes, and means for conducting the sheet formed in one pass into the other pass, said other pass being effective to combine the metal of said other batch with the metal of said sheet to form a sheet in said second pass, whereby said sheet contains metal from both said batches.

3. In the manufacture of sheet glass, means for maintaining two streams of molten metal, in combination with means operable periodically for dividing each of said streams into batches, two sheet forming passes, means for delivering batches from one of said streams to one of said passes, means for delivering batches from the other of said streams to the other of said passes, and

- means for conducting the comparatively thin sheet formed in one pass into the other pass, said other pass being effective to add metal from the other batch to form a comparatively thick sheet 5 containing metal from both said batches.
4. In the manufacture of sheet glass, means for maintaining two streams of molten metal, in combination with means operable periodically for dividing each of said streams into batches, and 10 means for forming said batches of metal into glass sheets so that the lower half of each sheet comprises a batch of metal from one stream and the upper half of each sheet comprises a batch of metal from the other stream.
- 15 5. The invention set forth in claim 4 in which means is provided for introducing reinforcing wire between said half sheets while they are being combined into a single sheet.
- 20 6. The invention set forth in claim 4 in which means is provided for laying reinforcing wire on the lower half sheet before it is covered by the upper half sheet, whereby said wire is embedded in the finished sheet.

25

80

7. In the manufacture of sheet glass, in combination, a refractory arch having a vertical opening through the crown thereof, means for maintaining a stream of molten metal downwardly through said opening, a ladle in the path of said stream, and means effective while said stream is flowing into said ladle for tilting said ladle to pour metal therefrom.

8. The invention set forth in claim 7 in which heat is supplied under said arch substantially as 85 described.

9. In the manufacture of sheet glass, in combination, a refractory arch having a vertical opening through the crown thereof, means for maintaining a stream of molten metal downwardly through said opening, a ladle in the path of said stream, a sheet-forming pass, and means effective 90 while said stream is flowing into said ladle for tilting said ladle to supply metal therefrom to said forming pass.

NICKLAS FRANZEN.

90

95

100

30

105

35

110

40

115

45

120

50

125

55

130

60

135

65

140

70

145

75

150